

Sept. 20, 1932.

J. B. WELLS ET AL

1,878,559

PROCESS OF MAKING CELLULOSIC FILMS

Filed June 4, 1928

Fig. 1.



Fig. 2.



Fig. 5.



Fig. 3.



Fig. 4.

Inventors  
Jackson B. Wells &  
Clarence L. A. Wynd,

By

M. M. Perrins  
Attorney

## UNITED STATES PATENT OFFICE

JACKSON B. WELLS AND CLARENCE L. A. WYND, OF ROCHESTER, NEW YORK, ASSIGNEES  
TO EASTMAN KODAK COMPANY, OF ROCHESTER, NEW YORK, A CORPORATION OF  
NEW YORK

## PROCESS OF MAKING CELLULOSIC FILMS

Application filed June 4, 1938. Serial No. 282,829.

This invention relates to processes for the manufacture of films and similar products, especially processes in which the films are set in liquid baths instead of by evaporation.

When film is formed by this method, which has certain inherent advantages, it has been found that there is a tendency to the production of a film surface that is not entirely smooth, but that has designs or patterns which tend to render the film unfit for use. We believe that this is caused by the solvents, after diffusion from the film being coagulated, as they stream along the surface of the partially formed film. These solvents, more or less dissolved in the aqueous bath, differentially attack the film, thus giving the striated markings.

The principal object of our invention is to overcome this and other defects and to produce a smooth highly polished surface on the film.

Various types of scrapers, squeegees, screens, sprays, etc., have been tried to overcome this inherent disadvantage in using the coagulation process and we have found that a submerged spray that immediately forces the diffused solvents from the film zone produces a film that is highly polished and is well suited to be used as a photographic support. Other types of liquid agitating means may be used,—for example, small propellers or other mechanical impellers rotating beneath the surface of the liquid. Of course, when this result is obtained by liquid coagulation in other than non-aqueous liquids, our submerged spray will work as advantageously.

The above and other objects may be accomplished by the process herein described, which may be carried out in the apparatus about to be described. This apparatus, it is to be understood, is merely illustrative.

Reference will now be made to the accompanying drawing in the several figures of which the same reference characters denote the same parts, and in which

Fig. 1 is a diagrammatic side elevation, partly in section, showing one form of apparatus in which our process may be carried out;

Fig. 2 is an elevation of a portion of the

spraying device in a plane parallel to the axis of the drum;

Fig. 3 is a diagram showing an alternative form of apparatus.

Figs. 4 and 5 show details of a modification. The viscous dope, after filtering, is poured into the elongated hopper 1. The lower part of this hopper is provided with accurately located edge pieces 2 and 3. By turning the screw 4, the thickness of the film 5 coated on the drum 8 from dope 6 in the hopper 1 may be controlled. Edge piece 2 projects slightly below edge piece 3, thus guiding a measured amount of dope 6 upon the drum 8, the outer surface of which is accurately polished. This cylinder rotates in a counter-clockwise direction, the sheet of dope passes into the chamber 9 which contains the coagulating liquid 10, which is fed into the liquid reservoir from the intake 11, passes countercurrent to the film sheet and out the exit pipe 12. While in chamber 9, the inequalities in the film gradually disappear, due to the force of gravity, and the film acquires a uniform thickness. After it is submerged in the liquid a fine spray of the coagulating liquid is forced against it from the spray pipes 13, which are provided with numerous fine perforations or nozzles. The liquid from the bottom of the liquid reservoir is drawn through the pipe 14 and the filter 15 by means of the centrifugal pump 16 from which it is fed through the pipe 17 to the spray nozzles in the pipe 13. The arrows 13a designate the flow of liquid from the spray to the film surface. As the film progresses through a bath, it gradually sets. It meets, as it advances, a coagulating liquid less concentrated in the film solvents and when it has traversed approximately three-quarters the circumference of the cylinder it is sufficiently strong to be removed therefrom over roller 18.

The formed film 20 may then pass through a suitable washing tank 30, and then through a drier 31. If desired, the air, rich in vaporized solvent from the drier, may pass through a scrubber 32 the water from which is used to fill the tank 30. These elements are merely indicated diagrammatically in Fig. 1.

Between the point that the film leaves the roll and dope is applied, any suitable cleaning and polishing means for reconditioning the drum may be inserted, such as the apparatus shown conventionally and described in U. S. Patent No. 1,187,299, Reid, June 20, 1916. A pipe 19' is provided with fine perforations in its underside through which water is sprayed upon the surface 7. This pipe 10 is parallel to the axis of the drum 8. The cleaning liquid is not allowed to flow down the surface 7 to the stripped film 20, or the bath 10, but is taken up by a dam in the shape of a hollow roll 21 having its periphery covered with a layer of soft rubber 22 through which a series of fine apertures are provided communicating to the center of the roll, the latter being connected to a vacuum apparatus, thus sucking the water through the dam 20 and out of the apparatus. The surface of the drum may be given a final conditioning by an absorbent roll 23, held against the surface by an adjustable spring 24.

Figure 2 illustrates one type of spray apparatus that may be used. The coagulating liquid is pumped into the spray at 19 and issued in a fine stream or spray from perforations or nozzles 28 uniformly distributed along the horizontal pipes.

Figure 3 is a diagrammatic view of an alternate method of agitating the liquid below the surface of the bath 10 by means of the banks of propellers 25 which are revolved by a gear train actuated by the power driven shaft 26.

It is preferable to have the spray totally submerged in order to keep the surface of the liquid bath quiet and free from agitation, otherwise the film will have undesirable markings, caused by this surface action. The spray, on the other hand, should not be too far below the surface or much of its effectiveness is lost. We have found that the spray should cover approximately one-third 45 of the area of the submerged film to insure optimum results.

It is desirable that the spray shall be as close to the surface as is possible without disturbance of the surface. The actual distance will depend on the particular material treated, the speed of the drum, the force of the spray and the other variable factors. If the surface is agitated, there is a tendency 55 for transverse markings to appear, as distinguished from those already described which are more or less longitudinal of the film.

One way to insure that the layer entering the bath will be free from disturbing surface irregularities of the bath is by providing a roller 35, as shown in Figure 4, which is spaced slightly from the layer 5 and is driven as indicated by the arrow, so that its surface 65 near the film moves in a direction op-

posite to the movement of the film, thus supporting a constant bead of liquid at 27.

In a modification shown in Figure 5, a roller 36 rests with slight pressure against the layer 5 at the point where it enters the bath 10 and is driven by its contact with the layer. It tends to smooth out irregularities in the surface of the layer.

We have further discovered that, in general, both kinds of markings are less if the air in chamber 9 is warmed and circulated gently through means of pipes 29, the action being apparently that there is a slight skinning over of the film surface prior to its reaching the setting bath proper.

This heated chamber is, therefore, useful in itself whether or not the submerged agitation is carried out.

Any suitable type of cellulosic dope or coagulating bath may be employed, such as are known in connection with the coagulation of viscose and cellulosic esters. As a typical example, may be mentioned nitrocellulose in a solution of methyl and butyl alcohol coagulated in an aqueous bath, such as described in the copending application of Jackson B. Wells, Serial No. 253,361, filed February 10, 1928. The apparatus herein described, except as otherwise specified, is of the type shown in said application, or it may be of the type shown in Reid Patent No. 1,187,929, June 20, 1916.

It is to be understood, however, that this process is general in its application to the formation of films, threads and the like, and is not confined to the specific materials and structure mentioned. We consider as within our invention all such modifications and equivalents as fall within the scope of the appended claim.

Having thus described our invention what we claim as new, and desire to secure by Letters Patent is,—

In the process of making smooth flexible films by the method in which a coagulable layer of cellulosic material is spread on a continuously moving smooth support, passed through a setting bath, and then stripped from said support in the form of a continuous band, and then passed through an aqueous bath and a drier in turn, the steps of recovering from the air of the drier vaporized solvents by means of a water scrubber and utilizing the water from the scrubber for the aqueous bath.

Signed at Rochester, New York, this 24th day of May, 1928.

JACKSON B. WELLS  
CLARENCE L. A. WYND.

125

130